

# UNITED STATES PATENT OFFICE.

ALBERT McGALL, OF NEW YORK, N. Y.

## METHOD OF PREPARING FINELY-DIVIDED METALS.

1,397,008.

Specification of Letters Patent. Patented Nov. 15, 1921.

No Drawing. Application filed September 16, 1918, Serial No. 254,346. Renewed February 2, 1921.  
Serial No. 442,012.

*To all whom it may concern:*

Be it known that I, ALBERT McGALL, a citizen of the United States, residing at New York, in the county of New York and State 5 of New York, have invented certain new and useful Improvements in Methods of Preparing Finely-Divided Metals, of which the following is a specification.

This invention is an electrolytic method 10 whereby oxidizable metals, such for example as zinc, copper, aluminum, etc., may be prepared in a state of minute subdivision but in non-oxidized condition. The metals so prepared are useful for a wide variety of 15 purposes, among which may be mentioned the preparation of electrodes for primary or secondary batteries, and the manufacture of explosives of the known type comprising a metallic component and an oxidizing agent, 20 such for example as ammonium nitrate.

I will describe my invention by reference to the preparation of non-oxidized zinc in minutely subdivided state, as a typical or illustrative example thereof. It will be 25 understood, however, that the invention is not restricted to the particular manipulative details below described, since the composition and concentration of the electrolyte, as well as the current conditions, may be 30 rather widely varied. Obviously also the conditions will be somewhat varied according to the particular metal which it is desired to obtain in subdivided form.

I prefer to proceed as follows:

35 Sheet zinc, which has preferably been amalgamated (although this is not essential) is coated by rubbing or otherwise with a thin layer of a suitable oleaginous substance, such for example as an organic or inorganic 40 (hydrocarbon) oil or grease, or material containing the same. The mineral grease known to the trade as "sponge grease", and having the characteristics of a non-flowing grease or oil, is entirely satisfactory for my pur- 45 poses.

The coated sheet is then connected as the anode in a suitable electrolyte, which is preferably acid, and may consist initially of a sulfuric acid solution having a specific gravity of about 1.3. A suitable cathode is provided which is preferably also of zinc: for although other metallic or conductive materials may be employed as cathode, there is less liability to loss of metal by local action 50 when zinc is used. Also, I prefer to apply a

like oleaginous coating to the cathode although this is not necessary for the practice of the invention. The coating of the cathode is, however, a distinct advantage for the reason that the cathode, if provided with an 60 oleaginous coating, is not acted upon by the electrolyte when the flow of current is interrupted.

Unidirectional current from an outside source is then caused to flow from the coated 65 sheet zinc as anode, whereupon, irrespective of the current density employed, a deposit of sponge or minutely subdivided zinc will be formed. This deposit is at most only loosely adherent to the cathode, and may be 70 either continuously or intermittently removed from the electrolyte, washed and dried. A current density of about one ampere per square inch of cathode surface will be found satisfactory; and the anode 75 and cathode areas may be substantially equal.

Contrary to what might be anticipated from the known insulating character of oleaginous materials, it will be found that 80 the coated metal, although quite unaffected by the acid electrolyte so long as no current flows through the system, nevertheless passes freely into solution as soon as current is applied from an external source, and is simultaneously deposited in minutely subdivided 85 or sponge form at the cathode. Instead, however, of forming a highly oxidizable, unstable, and often partially oxidized sponge, as is the case when the oleaginous coating is 90 omitted, the deposit will be found to be substantially non-oxidized, and relatively very stable. This I now attribute to the presence upon the individual particles of the deposit of an oleaginous protective coating of ex- 95 treme tenuity.

Finely subdivided copper is readily prepared under the above conditions. Metallic aluminum in minute subdivision may also be prepared in substantially the same manner. The aluminum deposit is however more liable to oxidation than zinc when removed from the solution, and especially when spread in contact with air. Consequently the aluminum deposit should preferably be shielded to 100 a reasonable degree from oxidizing influences, as for example by storing in an inert atmosphere, or even by compressing in order to reduce the exposed surface.

Metals which have been treated with an 110

oleaginous material and thereby rendered inactive toward acid electrolytes so long as no current flows through an electric circuit in which they may be included as anode, are 5 conveniently referred to as "immunized metals". The immunity from purely chemical as distinguished from electrochemical attack thus conferred is remarkably persistent; and, particularly in the case of electrodes which have been in use for some time, 10 may persist after thorough wiping of the electrode, and even after washing it with such cleansing agents as gasolene, etc., until all apparent traces of the oleaginous coating 15 have been removed. I employ the expression "immunized metal anode" in the claims to designate anodes possessing the above described characteristic due to the previous treatment with oil or equivalent material.

20 The term "metal" is used herein to include alloys, to which the method is likewise applicable.

I claim:—

1. Method of preparing oxidizable metals 25 in minutely subdivided, non-oxidized condition, comprising electrodepositing the metal in sponge form by means of an electric cur-

rent flowing from an immunized metal anode.

2. Method of preparing oxidizable metals 30 in minutely subdivided, non-oxidized condition, comprising electrodepositing the metal in sponge form by means of an electric current flowing from an anode of the same metal, said anode presenting surfaces having 35 an oleaginous coating.

3. Method of preparing oxidizable metals 40 in minutely subdivided, non-oxidized condition, comprising electrodepositing the metal in sponge form by means of an electric current passing between an anode and cathode of the desired metal, said anode immunized by treatment with an oleaginous substance.

4. Method of preparing oxidizable metals 45 in minutely subdivided, non-oxidized condition, comprising electrodepositing the metal in sponge form by means of an electric current passing between an anode and cathode of the desired metal, both of said electrodes immunized by treatment with an oleaginous 50 substance.

In testimony whereof, I affix my signature.

ALBERT McGALL.